



US005221296A

# United States Patent [19]

Schwerzel et al.

[11] Patent Number: 5,221,296

[45] Date of Patent: Jun. 22, 1993

## [54] ABRASIVES

[75] Inventors: Thomas Schwerzel, Meckenheim; Kurt Wendel, Ludwigshafen; Hermann Rockstroh, Maxdorf, all of Fed. Rep. of Germany

[73] Assignee: BASF Aktiengesellschaft, Ludwigshafen, Fed. Rep. of Germany

[21] Appl. No.: 957,168

[22] Filed: Oct. 7, 1992

## [30] Foreign Application Priority Data

Oct. 7, 1991 [DE] Fed. Rep. of Germany ..... 4133191

[51] Int. Cl. 5 ..... C09K 3/14

[52] U.S. Cl. ..... 51/298

[58] Field of Search ..... 51/298

## [56] References Cited

## U.S. PATENT DOCUMENTS

4,350,498 9/1982 Zimmer ..... 51/298

4,652,274 3/1987 Boettcher et al. ..... 51/298

4,690,692 9/1987 Hesse et al. ..... 51/298

4,773,920 9/1988 Chrisman et al. ..... 51/298

5,055,113 10/1991 Larson et al. ..... 51/298

## FOREIGN PATENT DOCUMENTS

0261098 3/1988 European Pat. Off. .

*Primary Examiner*—Mark L. Bell*Assistant Examiner*—Willie J. Thompson*Attorney, Agent, or Firm*—Oblon, Spivak, McClelland, Maier & Neustadt

## [57] ABSTRACT

Abrasives based on finely divided abrasive particles bonded to one another and/or to a support by means of a binder, where the binder is the solid component of an aqueous polymer dispersion which is obtainable by polymerizing unsaturated monomers which can be polymerized by means of free radicals, in the aqueous phase in the presence of a monosaccharide, oligosaccharide, polysaccharide, oxidatively, hydrolytically and/or enzymatically degraded polysaccharide, chemically modified monosaccharide, oligosaccharide or polysaccharide, or a mixture of the said compounds, by the process of free-radical aqueous emulsion polymerization.

2 Claims, No Drawings

## ABRASIVES

The present invention relates to abrasives based on finely divided abrasive particles bonded to one another and/or to a support by means of a binder, where the binder is the solid component of an aqueous polymer dispersion which is obtainable by polymerizing unsaturated monomers which can be polymerized by means of free radicals, in the aqueous phase in the presence of a monosaccharide, oligosaccharide, polysaccharide, oxidatively, hydrolytically and/or enzymatically degraded polysaccharide, chemically modified monosaccharide, oligosaccharide or polysaccharide, or a mixture of the said compounds, by the process of free-radical aqueous emulsion polymerization.

EP-A 261 098 discloses abrasives whose abrasive particles are bonded to a radiation-curable polymeric binder in order to achieve satisfactory properties. The requirement for radiation curing is disadvantageous.

It is an object of the present invention to provide entirely satisfactory abrasives based on polymeric binders which do not require radiation curing.

We have found that this object is achieved by the abrasives defined at the outset.

Particularly suitable finely divided abrasive particles are fused or sintered corundum, zirconium corundum, silicon carbide and emery. Suitable support materials include flexible substrates, e.g. paper, vulcanized fiber, woven fabrics, knitted fabrics, nonwovens based on natural and/or synthetic fibers, plastic films or metal foils.

Suitable monomers which can be polymerized by means of free radicals include, in particular, monoethylenically unsaturated monomers, such as olefins, e.g. ethylene, vinylaromatic monomers, such as styrene,  $\alpha$ -methylstyrene,  $\alpha$ -chlorostyrene and vinyltoluenes, vinyl and vinylidene halides, such as vinyl chloride and vinylidene chloride, esters made from vinyl alcohol and monocarboxylic acids having 1 to 18 carbon atoms, such as vinyl acetate, vinyl propionate, vinyl n-butyrate, vinyl laurate and vinyl stearate, esters made from  $\alpha$ , $\beta$ -monoethylenically unsaturated mono- and dicarboxylic acids, preferably having 3 to 6 carbon atoms, such as, in particular, acrylic acid, methacrylic acid, 45 maleic acid, fumaric acid and itaconic acid, with alkanols generally having from 1 to 12, preferably from 1 to 8, in particular from 1 to 4, carbon atoms, such as, in particular, methyl, ethyl, n-butyl, isobutyl and 2-ethylhexyl acrylates and methacrylates, dimethyl maleate and n-butyl maleate, nitriles of  $\alpha$ , $\beta$ -monoethylenically unsaturated carboxylic acids, such as acrylonitrile, and C.: conjugated dienes, such as 1,3-butadiene and isoprene. Said monomers are essentially insoluble in aqueous media and generally form the principal monomers, 55 which normally make up a proportion of greater than 50% by weight, based on the total amount of monomers to be polymerized. Monomers which, when polymerized alone, usually give homopolymers of increased water solubility are normally only copolymerized as modifying monomers in amounts, based on the total amount of monomers to be polymerized, of less than 50% by weight, in general from 0.5 to 20% by weight, preferably from 1 to 10% by weight.

Examples of such monomers are  $\alpha$ , $\beta$ -monoethylenically unsaturated mono- and dicarboxylic acids having 3 to 6 carbon atoms, and amides thereof, e.g. acrylic acid, methacrylic acid, maleic acid, fumaric acid, ita-

conic acid, acrylamide and methacrylamide, furthermore vinylsulfonic acid and water-soluble salts thereof, and N-vinylpyrrolidone. Monomers which usually increase the intrinsic strength of films formed by the aqueous polymer dispersion are generally likewise only copolymerized in minor amounts, usually from 0.5 to 10% by weight, based on the total amount of monomers to be polymerized. Such monomers normally contain an epoxide, hydroxyl, N-methylol or carbonyl group or at least two non-conjugated ethylenically unsaturated double bonds. Examples of this are N-alkylolamides of  $\alpha$ , $\beta$ -monoethylenically unsaturated carboxylic acids having 3 to 10 carbon atoms and esters thereof with alcohols having 1 to 4 carbon atoms, of which N-methylolacrylamide and N-methylolmethacrylamide are very particularly preferred, monomers containing two vinyl radicals, monomers containing two vinylidene radicals, and monomers containing two alkenyl radicals. Particularly suitable here are diesters of dihydric alcohols with  $\alpha$ , $\beta$ -monoethylenically unsaturated monocarboxylic acids, of which in turn acrylic acid and methacrylic acid are preferably employed. Examples of such monomers containing two non-conjugated ethylenically unsaturated double bonds are alkylene glycol diacrylates and dimethacrylates, such as ethylene glycol diacrylate, 1,3-butylene glycol diacrylate, 1,4-butylene glycol diacrylate and propylene glycol diacrylate, divinylbenzene, vinyl methacrylate, vinyl acrylate, allyl methacrylate, allyl acrylate, diallyl maleate, diallyl fumarate and methylenebisacrylamide. In addition to monomers containing unsaturated double bonds, it is also possible to copolymerize minor amounts, usually from 0.01 to 4% by weight, based on the monomers to be polymerized, of molecular weight regulators, such as tert-dodecyl mercaptan. Such substances are preferably added to the polymerization zone in a mixture with the monomers to be polymerized.

Preferred classes of aqueous polymer dispersions to be employed according to the invention are those whose polymers are obtainable by free-radical polymerization of monomer mixtures which comprise

from 50 to 100% by weight of esters of acrylic and/or methacrylic acid with alkanols having 1 to 12 carbon atoms and/or styrene (class I) or

from 70 to 100% by weight of styrene and/or butadiene (class II) or

from 70 to 100% by weight of vinyl chloride and/or vinylidene chloride (class III),

class I being particularly preferred and preferably covering the following monomer compositions:

from 90 to 99% by weight of esters of acrylic and/or methacrylic acid with alkanols having 1 to 8 carbon atoms and/or styrene, and

from 1 to 10% by weight of acrylic acid, methacrylic acid or a mixture thereof.

Of very particular interest are the following monomer compositions:

from 90 to 99% by weight of n-butyl acrylate and/or styrene,

from 1 to 10% by weight of acrylic acid and/or methacrylic acid.

Said monomers are polymerized according to the invention by free-radical aqueous emulsion polymerization in the presence of polysaccharides, oligosaccharides, monosaccharides and/or derivatives thereof. They may be of vegetable or animal origin, soluble in water or only dispersible therein. Suitable compounds include swollen starches, which are obtainable, for ex-

ample, by hydrothermal treatment of native starch. Soluble starches are furthermore suitable. These are starches which have been slightly degraded by means of acids or enzymes or have been oxidized by means of mild oxidants, and, even in relatively high concentrations, do not give viscous pastes on boiling with water, but instead give relatively thin liquids. Also suitable are acid-modified starches obtained by warming an aqueous starch suspension at below the gelatinization temperature in the presence of small amounts of acid. Also 10 suitable are oxidatively modified starches. Examples of oxidants which can be used are chromic acid, permanganate, hydrogen peroxide, nitrogen dioxide, hypochlorite and periodic acid. Suitable starting starches are in principle all native starches, such as cereal starches (e.g. corn, wheat, rice or millet), tuber and root starches (e.g. potatoes, tapioca root or arrowroot) or sago starches. It is particularly advantageous to use roast dextrans, as described, for example, in EP-A 408 099 and EP-A 334 15 515. They can be obtained by heating moist-dry starch, usually in the presence of small amounts of acid. Examples of typical roast dextrans are the commercially available white and yellow dextrans, and furthermore the dextrans marketed under the trade names Noredux® and Tackidex®. The term dextrin here is used very 20 generally for starch degradation products. However, it is very particularly advantageous to carry out the free-radical emulsion polymerization in the presence of sugared starches. These are starch degradation products obtainable by hydrolysis in the aqueous phase and preferably having a weight average molecular weight  $M_w$  of from 2500 to 25000. Details on the preparation of said starches and starch derivatives are given in G. Tegge, Stärke und Stärkederivate, Behr's Verlag, Hamburg, 1984. It is of course possible to carry out the invention 25 using said starches and starch derivatives in chemically modified form, for example modified by etherification or esterification.

This chemical modification can be carried out on the starting starch even before its degradation or thereafter. Esterification reactions are possible using either inorganic or organic acids, or the anhydrides or chlorides thereof. Of particular interest are phosphated and acetylated derivatives. The most common etherification method is treatment with organic halogen compounds, 30 epoxides or sulfates in aqueous alkaline solution. Particularly suitable ethers are alkyl ethers, hydroxyalkyl ethers, carboxyalkyl ethers and allyl ethers. Also suitable are cyanoalkylated derivatives and products of the reaction with 2,3-epoxypropyltrimethylammonium chloride. Chemically unmodified products are preferred. Of course, monosaccharides and oligosaccharides and products of the degradation of cellulose, for 35 example cellobiose and oligomers thereof, are also suitable.

The sugared starches having a weight average molecular weight of from 2500 to 25000 very particularly preferably to be used according to the invention are commercially available as such (for example the C\* PUR Products 01906, 01908, 01910, 01912, 01915, 40 01921, 01924, 01932 and 01934 from Cerestar Deutschland GmbH, D-1150 Krefeld 12). Sugared starches of this type differ chemically from roast dextrans through the fact, inter alia, that recombination and branching are essentially impossible, evident not least in different molecular weight distributions, on hydrolytic degradation in an aqueous medium (usually suspensions or solutions), which is generally carried out at solids contents

of from 10 to 30% by weight and preferably with acid or enzyme catalysis. Thus, sugared starches which have a bimodal molecular weight distribution have proven particularly advantageous according to the invention. 5 The preparation of sugared starches is generally known and is described, inter alia, in G. Tegge, Stärke und Stärkederivate, Behr's Verlag, Hamburg 1984, p. 173 and p. 220 ff. and in EP-A 441 197. The sugared starches to be used according to the invention are preferably those whose weight average molecular weight  $M_w$  is in the range from 4000 to 16000, particularly preferably in the range from 6500 to 13000.

The sugared starches to be used according to the invention are normally completely soluble in water at 15 room temperature, the solubility limit generally being above 50% by weight, which proves particularly advantageous for the preparation of the aqueous polymer dispersions according to the invention.

It has furthermore proven favorable for the sugared starches to be used according to the invention to have a nonuniformity  $U$  (defined as the ratio between the weight average molecular weight  $M_w$  and the number average molecular weight  $M_n$ ;  $U$  characterizes the molecular weight distribution) in the range from 6 to 12.  $U$  is particularly advantageously from 7 to 11 and very particularly advantageously from 8 to 10.

It is furthermore advantageous for the proportion by weight of the sugared starches having a molecular weight of below 1000 to be used according to the invention to be at least 10% by weight, but not more than 70% by weight. This proportion by weight is particularly preferably in the range from 20 to 40% by weight.

It is furthermore advisable to use sugared starches to be used according to the invention whose dextrose equivalent DE is from 5 to 40, preferably from 10 to 30, particularly preferably from 10 to 20. The DE value characterizes the reduction capacity, relative to the reduction capacity of anhydrous dextrose, and is determined in accordance with DIN 10308, Edition 5.71, produced by the German Standards Committee on Foodstuffs and Agricultural Products (cf. also Günther Tegge, Stärke und Stärkederivate, Behr's Verlag, Hamburg 1984, p. 305).

It has also been found that aqueous polymer dispersions which have a particularly favorable property profile are obtained if sugared starches to be used according to the invention are used whose 40% strength by weight aqueous solutions have a dynamic viscosity  $\eta^{40}$  [Pa.s], determined in accordance with DIN 53 019 at 25° C. and a shear gradient of 75 s., of from 0.01 to 0.06, 45 preferably from 0.015 to 0.04, particularly preferably from 0.02 to 0.035.

It should be noted at this point that molecular weight data for saccharides and derivatives thereof to be used according to the invention are based in this publication, unless expressly stated otherwise, on determinations by means of gel permeation chromatography, carried out under the following conditions:

|                 |                                                                                                              |
|-----------------|--------------------------------------------------------------------------------------------------------------|
| Columns:        | 3 steel units measuring 7.5 x 600 mm, filled with TSK gel G 2000 PW; G 3000 PW and G 4000 PW. Mesh 5 $\mu$ m |
| Eluent:         | Distilled water.                                                                                             |
| Temp.:          | RT (room temperature)                                                                                        |
| Detection:      | Differential refractometer (for example ERC 7511)                                                            |
| Flow rate:      | 0.8 ml/min., pump (for example ERC 64.00)                                                                    |
| Injection vol.: | 20 $\mu$ l, valve (for example VICI 6-way valve)                                                             |

-continued

|              |                                                                                                                                                                                                                         |
|--------------|-------------------------------------------------------------------------------------------------------------------------------------------------------------------------------------------------------------------------|
| Evaluation:  | Bruker Chromstar GPC software                                                                                                                                                                                           |
| Calibration: | The calibration was carried out in the low-molecular-weight range using glucose, raffinose, maltose and maltopentose. For the higher-molecular-weight range, pullulan standards having a polydispersity <1.2 were used. |

The monosaccharides, oligosaccharides and polysaccharides and/or derivatives thereof present according to the invention during the free-radical aqueous emulsion polymerization may be present either as the only dispersants or in a mixture with other surfactants. If they are employed as the only dispersants, they are normally present in the aqueous polymer dispersions according to the invention in amounts of from 1 to 120% by weight, based on the amount of monomers to be polymerized.

Suitable secondary surfactants are in principle the protective colloids and emulsifiers otherwise usually employed as dispersants. A detailed description of suitable protective colloids is given in Houben-Weyl, Methoden der organischen Chemie, Volume XIV/1, Makromolekulare Stoffe, Georg-Thieme-Verlag, Stuttgart, 1961, pp. 411 to 420. Suitable secondary emulsifiers are anionic, cationic and nonionic emulsifiers. It is preferred for the secondary surfactants to be exclusively emulsifiers, whose relative molecular weights, in contrast to the protective colloids, are usually below 2000. It is of course necessary, if mixtures of surfactants are used, for the individual components to be compatible with one another, which can be checked in case of doubt by means of a few preliminary experiments. The secondary surfactants used are preferably anionic and nonionic emulsifiers. Examples of customary secondary emulsifiers are ethoxylated fatty alcohols (degree of ethoxylation from 3 to 50, C<sub>8</sub>— to C<sub>36</sub>-alkyl radical), ethoxylated mono-, di- and trialkylphenols (degree of ethoxylation from 3 to 50, C<sub>4</sub>— to C<sub>9</sub>-alkyl radical), alkali metal salts of dialkyl esters of sulfosuccinic acid and alkali metal and ammonium salts of alkyl sulfates (C<sub>8</sub>— to C<sub>12</sub>-alkyl radical), of ethoxylated alkanols (degree of ethoxylation from 4 to 30, C<sub>12</sub>— to C<sub>18</sub>-alkyl radical), of ethoxylated alkylphenols (degree of ethoxylation from 3 to 50, C<sub>4</sub>— to C<sub>9</sub>-alkyl radical), of alkylsulfonic acids (C<sub>12</sub>— to C<sub>18</sub>-alkyl radical) and of alkylarylsulfonic acids (C<sub>9</sub>— to C<sub>18</sub>-alkyl radical). Further suitable emulsifiers are given in Houben-Weyl, Methoden der organischen Chemie, Volume XIV/1, Makromolekulare Stoffe, Georg Thieme Verlag, Stuttgart, 1961, pages 192 to 208. Secondary surfactants are generally used in amounts of up to 5% by weight, based on the amount of monomers to be polymerized.

The emulsion polymerization temperature is generally from 30° to 95° C., preferably from 75° to 90° C. The polymerization medium may either comprise water alone or a mixture of water and water-miscible liquids, such as methanol. It is preferred to use water alone. The emulsion polymerization can be carried out either as a batch process or in the form of a feed process, including a step or gradient procedure. Preference is given to the feed process, in which part of the polymerization batch is heated to the polymerization temperature and partially polymerized, and the remainder of the polymerization batch is subsequently fed to the polymerization zone continuously, in steps or with superposition of a concentration gradient, usually via a plurality of spatially separate feed streams, of which one or more con-

tain the monomers in pure or emulsified form, while maintaining the polymerization. In an applicationally advantageous manner, the initially introduced mixture and/or the monomer feed stream contains small amounts of emulsifiers, generally less than 0.5% by weight, based on the total amount of monomers to be polymerized, in order to reduce the surface tension of the dispersion medium and thus to simplify stirring in. The monomers are therefore frequently fed to the polymerization zone after preemulsification with these assistant emulsifiers. It is advantageous for all the monosaccharide, oligosaccharide or polysaccharide and/or derivatives thereof to be present in an aqueous mixture.

Suitable free-radical polymerization initiators are all those which are capable of initiating a free-radical aqueous emulsion polymerization. These may be either peroxides, for example alkali metal peroxydisulfates or H<sub>2</sub>O<sub>2</sub>, or azo compounds.

Also suitable are combined systems comprising at least one organic reducing agent and at least one peroxide and/or hydroperoxide, e.g. tert-butyl hydroperoxide and the sodium metal salt of hydroxymethanesulfonic acid or hydrogen peroxide and ascorbic acid. Also suitable are combined systems additionally containing a small amount of a metal compound which is soluble in the polymerization medium and whose metallic component can exist in more than one oxidation state, e.g. ascorbic acid/iron(II) sulfate/hydrogen peroxide, where ascorbic acid is also frequently replaced by the sodium metal salt of hydroxymethanesulfonic acid, sodium sulfite, sodium hydrogen sulfite or sodium metal bisulfite and hydrogen peroxide is frequently replaced by tert-butyl hydroperoxide or alkali metal peroxydisulfates and/or ammonium peroxydisulfates. In the combined systems, it is furthermore expedient to use the sugared starches as the reducing component. In general, the amount of free-radical initiator systems employed is from 0.1 to 2% by weight, based on the total amount of the monomers to be polymerized. Particularly preferred initiators are ammonium and/or alkali metal peroxydisulfates, alone or as a constituent of combined systems. Particular preference is given to sodium peroxydisulfate.

The manner in which the free-radical initiator system is added to the polymerization reactor during the free-radical aqueous emulsion polymerization according to the invention is of somewhat secondary importance. It can either all be introduced into the polymerization reactor at the beginning, or added continuously or stepwise as it is consumed during the free-radical aqueous emulsion polymerization. In detail, this depends in a manner known to an average person skilled in the art both on the chemical nature of the initiator system and on the polymerization temperature. In a preferred procedure, some is introduced at the beginning and the remainder is added to the polymerization zone as it is consumed.

It is of course also possible to carry out the free-radical aqueous emulsion polymerization according to the invention under superatmospheric or reduced pressure.

The aqueous polymer dispersions according to the invention are generally prepared with total solids contents of from 15 to 65% by weight, particular preference being given, for application reasons, to those which contain from 10 to 75% by weight, very particularly preferably from 20 to 60% by weight, based on the monomers to be polymerized, of monosaccharides, oli-

gosaccharides or polysaccharides to be used according to the invention, and/or derivatives thereof.

Binders for abrasive particles which are suitable in a very particularly advantageous manner for the production of abrasives are aqueous polymer dispersions according to the invention whose polymers are obtainable by free-radical polymerization of monomer mixtures which have the following monomer composition, comprising

from 39 to 69% by weight of at least one ester of  $\alpha,\beta$ -monoethylenically unsaturated mono- and di-carboxylic acids having 3 to 6 carbon atoms with alkanols having 1 to 6 carbon atoms (monomers a), from 30 to 60% by weight of styrene (monomer b), from 1 to 10% by weight of at least one monomer

from the group comprising  $\alpha,\beta$ -monoethylenically unsaturated carboxylic acids having 3 to 6 carbon atoms, and amides and nitriles thereof, (monomers c) and

from 0 to 10% by weight of one or more monomers from the group comprising N-alkylolamides of  $\alpha,\beta$ -monoethylenically unsaturated carboxylic acids having 3 to 6 carbon atoms, with 1 to 4 carbon atoms in the alkyl group, and monomers having up to 25 carbon atoms and containing two non-conjugated, ethylenically unsaturated double bonds (monomers d),

and which contain, based on the monomers to be polymerized, from 1 to 120% by weight, preferably from 10 to 65% by weight, particularly preferably from 35 to 55% by weight, of monosaccharide, oligosaccharides or polysaccharides and/or derivatives thereof. It is of course possible for all or some of the monomers d to be replaced by other crosslinking monomers mentioned in this publication.

Conversion of the abrasive particles to abrasives can be carried out, for example, by mixing the finely divided abrasive particles with the aqueous polymer dispersions to be used according to the invention while establishing the desired binder content, in general (calculated in dry form) from 0.1 to 10% by weight, based on the amount of finely divided starting material, shaping the mixture, if desired after adding known assistants, if desired compacting the material by exerting pressure, and subsequently curing the material.

Abrasives according to the invention are preferably produced by first applying to the support a so-called make coat, into which, in the wet state, the abrasive particles are embedded. After a first fixing of the abrasive particles by drying (curing), a second, so-called size coat is generally applied in order to improve the embedding and fixing of the particles. In principle, the make coat and size coat can comprise different binders. According to the invention, at least one of the two, preferably the size coat and particularly preferably both, comprise the aqueous polymer dispersions according to the invention.

It is noteworthy that, on use of the aqueous polymer dispersions according to the invention, which are usually used for this purpose with a total solids content of from 40 to 60% by weight, the curing process does not necessarily require the use of elevated temperatures (normally from 50° to 250° C.), but thorough curing also takes place at a satisfactory rate when left to itself at room temperature. The curing can also be achieved in an applicationally particularly elegant manner by exposing the material to be cured to the action of microwaves. In this respect, aqueous polymer dispersions

according to the invention which are obtainable by free-radical aqueous emulsion polymerization of mixtures of monomers a, b, c and d whose monomer composition is selected so that a polymer built up only from monomers a, b and c would have a glass transition temperature in the range from 0° to 40° C., are recommended with particular advantage.

According to Fox (T. G. Fox, Bull. Am. Phys. Soc. (Ser. II) 1 (1956) 123), the glass transition temperature of copolymers is given, to a close approximation, by:

$$\frac{1}{T_g} = \frac{X^1}{T_g^1} + \frac{X^2}{T_g^2} + \dots + \frac{X^s}{T_g^s}$$

where  $X^1, X^2, \dots, X^s$  denote the proportions by weight of monomers 1, 2, ..., s, and  $T_g^1, T_g^2, \dots, T_g^s$  denote the glass transition temperatures of the respective polymers built up only from one of the monomers 1, 2, ..., s, in Kelvin. The glass transition temperatures of the monomers a, b and c are essentially known and are listed, for example, in J. Brandrup, E. H. Immergut, Polymer Handbook, 1st Edn., J. Wiley, New York 1966, and 2nd Edn., J. Wiley, New York 1975.

Typical requirements made of binders suitable for the production of abrasives are:

good adhesion, both to the substrate and to the abrasive particles,  
curable rapidly under gentle conditions,  
very low loading of the support material,  
high heat distortion resistance,  
increased flowability on application, and  
good mechanical properties during grinding (formation of hard, tough films).

These requirements are achieved entirely satisfactorily by the aqueous polymer dispersions according to the invention. Thus, curing when they are used does not necessarily require elevated temperatures, but can be carried out at room temperature and particularly advantageously under the action of microwaves. This is particularly gentle for the support material and avoids extreme removal of water, which makes complex regeneration of the carrier material in climatic zones unavoidable.

Their variable flow behavior proves to be particularly advantageous if the aqueous polymer dispersions according to the invention are used as a size coat, since it enables the binder to penetrate into the interstices between the abrasive particles.

In addition, the binders according to the invention are distinguished, in particular, by increased heat distortion resistance, so that the abrasive particles remain fixed in their position even at the temperatures (150° C. or more) which occur during grinding. Loosening of the abrasive particles (which reduces the grinding effect) or even dislodgement is thus suppressed. The make coat is usually applied in a dry film thickness of from 10 to 100  $\mu\text{m}$  and the size coat in a dry film thickness of from 20 to 10<sup>3</sup>  $\mu\text{m}$ .

If the polymers also contain incorporated monomers d, particularly high heat distortion resistances result. In addition, the heat distortion resistances can be further increased by adding up to 20% by weight, based on the polymerized monomers, of saturated dialdehydes, preferably those of the formula I



(i)

before the aqueous polymer dispersions to be used according to the invention are used, dialdehydes of the formula I where  $n=0$  to 2 being preferred. Other suitable additives for increasing the heat distortion resistance are condensation products based on formaldehyde, melamine, phenol and/or urea, eg. Urecoll ® 118. The amounts to be used can be up to 250% by weight, based on the solids content of the aqueous polymer dispersions according to the invention determined 15 without the sugared starch.

However, the last-mentioned additives only have an advantageous effect in the manner described if the curing is carried out at elevated temperature, in general from 100° to 250° C., or in the presence of acid. The latter can be achieved in a simple manner by adjusting the pH of the dispersion medium of the aqueous polymer dispersions to be used according to the invention to from 1 to 5, preferably to from 2 to 3. If heat distortion resistances within usual limits are required, it is preferred to use no additives. 25

### EXAMPLES

#### 1. Preparation of aqueous polymer dispersions to be used according to the invention

A mixture of

400 g of water,

200 g of sugared starch C\* PUR 01910

71 g of feed 1 and

10 g of feed 2

35 was heated to 85° C. and kept at this temperature for 15 minutes. The remainders of feeds 1 and 2 were subsequently fed continuously to the polymerization zone beginning at the same time (feed 1 over the course of 2.5 hours, feed 2 over the course of 3 hours) while maintaining the temperature of 85° C. The mixture was subsequently polymerized for a further hour (85° C.) and then cooled to room temperature. The total solids content of the resultant aqueous polymer dispersion was about 50% by weight. 45

|         |                           |
|---------|---------------------------|
| Feed 1: | 250 g of n-butyl acrylate |
|         | 225 g of styrene          |
|         | 25 g of acrylic acid      |

50

preemulsified in 204 g of water by means of 0.5 g of the sodium salt of dodecylbenzenesulfonic acid.

|         |                                                              |
|---------|--------------------------------------------------------------|
| Feed 2: | 2.5 g of sodium peroxydisulfate dissolved in 100 g of water. |
|---------|--------------------------------------------------------------|

55

#### 2 Abrasive articles based on finely divided abrasive particles bound to a support by means of an aqueous polymer dispersion according to the invention

100 g of various aqueous polymer dispersions according to the invention, prepared as in Example 1 and to some of which 0.062 part by weight of glyoxal had been added per part by weight of sugared starch present, 65 were mixed with 1 g of Lumiten ® (wetting agent) and applied to a base paper at an application rate of 20 g/m<sup>2</sup> (dry). Semiprecious corundum 60 was scattered into the

wet coating, and the paper coated in this way was dried at 90° C. for 3 minutes. The same binder was subsequently applied at an application rate of 60 g/m<sup>2</sup> (dry) as the size coat and likewise dried (30 minutes). The abrasive paper obtainable in this way was tested by means of an APG 100/20 abrasion tester (Maag & Schank, Gomaringen). The test specimens used were rigid PVC test specimens measuring 40 mm × 20 mm × 5 mm. In this test, an area of 20 mm × 5 mm was rubbed off using 500 strokes (load 1 kg), with the abrasive paper being moved to and fro beneath the test specimen for a length of 10.5 cm. The abrasion, defined as follows, is used as a measure of the quality of the binder:

$$\text{Abrasion [\%]} = \frac{\text{Weight of test specimen before testing} - \text{Weight of test specimen after testing}}{\text{Weight of test specimen before testing}} \times 100$$

The Table shows the results.

TABLE

| Binder | Glyoxal | Drying temperature (°C.) |               |
|--------|---------|--------------------------|---------------|
|        |         | Size coat                | Abrasion [\%] |
| Ex. 1  | —       | 90                       | 8.7           |
| Ex. 1  | +       | 90                       | 10.7          |
| X      | +       | 150                      | 7             |
| Y      | +       | 150                      | 7.5           |

30 X and Y prepared as in Example 1, but with a different monomer composition;

|    |                                                                                                         |
|----|---------------------------------------------------------------------------------------------------------|
| X: | 50% by weight of n-butyl acrylate,<br>45% by weight of styrene and<br>5% by weight of methacrylic acid; |
| Y: | 50% by weight of n-butyl acrylate,<br>40% by weight of styrene and<br>10% by weight of acrylic acid.    |

40 If C\*PUR 01910 is replaced by C\*PUR 01906, 01908, 01912, 01915, 01921, 01924, 01932 or 01934, results of the same order of magnitude were obtained. C\*PUR 01910 and 01915 proved to be particularly advantageous. The sugared starches mentioned can be characterized as follows:

| Type  | $M_w$       | U       | % by weight<br><1000 | DE    | $\eta^{40}$<br>[Pa · s] |
|-------|-------------|---------|----------------------|-------|-------------------------|
| 01906 | 20080       | 10.9    | 12.2                 | 2-5   | —                       |
| 01908 | 19290       | 10.0    | 15.9                 | 8-10  | 0.056                   |
| 01910 | 10540-12640 | 8.5-9.9 | 24.7-26.4            | 11-14 | 0.030                   |
| 01915 | 6680-8350   | 6.8-8.4 | 32.9-34.7            | 17-19 | 0.021                   |
| 01921 | 6700        | 7.4     | 39.1                 | 20-23 | 0.017                   |
| 01924 | 4730        | 6.8     | 53.6                 | 26-30 | 0.014                   |
| 01932 | 4500        | 7.9     | 63.2                 | 33-35 | 0.011                   |
| 01934 | 3000        | 6.0     | 68.4                 | 36-39 | 0.009                   |

60 Determination of  $M_w$  by vapor pressure osmometry gave the following values for the preferred types 01910 and 01915:

1560 g/mol (1910)

980 g/mol (1915)

We claim:

1. An abrasive based on finely divided abrasive particles bonded to one another and/or to a support by means of a binder, where the binder is the solid component of an aqueous polymer dispersion which is obtainable by polymerizing unsaturated monomers which can

be polymerized by means of free radicals, in the aqueous phase in the presence of a monosaccharide, oligosaccharide, polysaccharide, oxidatively, hydrolytically and/or enzymatically degraded polysaccharide, chemically modified monosaccharide, oligosaccharide or polysaccharide, or a mixture of the said compounds, by the process of free-radical aqueous emulsion polymerization.

2. An abrasive as claimed in claim 1, whose binder is obtainable by free-radical polymerization of monomer

mixtures comprising the following monomer composition:

from 39 to 69% by weight of at least one ester of  $\alpha,\beta$ -monoethylenically unsaturated mono- and di-carboxylic acids having 3 to 6 carbon atoms with alkanols having 1 to 6 carbon atoms,  
 from 30 to 60% by weight of styrene,  
 from 1 to 10% by weight of at least one monomer from the group consisting of  $\alpha,\beta$ -monoethylenically unsaturated carboxylic acids having 3 to 6 carbon atoms, and amides and nitriles thereof, and from 0 to 10% by weight of crosslinking monomers.

\* \* \* \* \*

15

20

25

30

35

40

45

50

55

60

65